

June 8, 1943.

P. GOLDFINGER  
COLOR PHOTOGRAPHIC MATERIAL AND  
METHOD OF USING THE SAME  
Filed Dec. 4, 1939

2,321,195



By *F. Gerald Toye*  
Attorney

## UNITED STATES PATENT OFFICE

2,321,195

COLOR PHOTOGRAPHIC MATERIAL AND  
METHOD OF USING THE SAME

Paul Goldfinger, Brussels-Uccle, Belgium, assignor, by mesne assignments, to Chromogen, Incorporated, a corporation of Nevada

Application December 4, 1939, Serial No. 307,507  
In Great Britain December 22, 1938

12 Claims. (Cl. 95—6)

In many of the known processes, photographic dye pictures are obtained by exposing a layer of light-sensitive silver halide emulsion and converting the latent images thus produced, or the silver images formed by developing, or even the unexposed silver halide that has been unaffected by the developing process into a dye picture. It is desirable and necessary in every instance in order to ensure the greatest fidelity in the reproduction of the objects photographed, that the graduations of the dye picture subsequently obtained correspond as far as possible with the graduations of light i. e., range of light intensities originally recorded in the silver halide emulsion during the exposure.

It has, however, been found that generally the hues of the dye picture correspond to the graduations of light or range of light intensities recorded during the exposure to only a limited extent and that, for instance, when a silver image in which there are 15 graduations of silver densities is processed to obtain a dye picture, there are but 8 graduations of hue to be clearly distinguished in the latter; the densest graduations in the silver image are not reproduced by distinct variations in the dye picture. Taking as an example the case of a dye picture obtained by local destruction of the dye at the silver areas in a uniformly colored layer, it will be found that the dye is totally destroyed or its density is uniformly reduced at the places where the silver deposit is greatest without regard to the different graduations of the silver deposit and thus the graduations of the darkest areas are not reproduced by the dye picture.

The invention, both as to its organization and method of operation, together with additional objects and advantages thereof, will best be understood from the following description of specific embodiments when read in connection with the accompanying drawing, in which like reference characters indicate like parts throughout.

Fig. 1 is a diagrammatic view in cross-section of a diffusely dyed layer which has been exposed and the silver image developed;

Fig. 2 is a diagrammatic view in cross-section of the layer shown in Fig. 1 after the silver image has been transposed to a dye image;

Fig. 3 is a diagrammatic view in cross-section of a layer similar to that shown in Fig. 2 containing a dye image of greater detail than that in Fig. 2;

Fig. 4 is a diagrammatic view in cross-section of a two-layer element comprising layers of the type shown in Figs. 1 and 3, both of which layers

have been diffusely dyed the same color and have been exposed and the silver images developed;

Fig. 5 is a diagrammatic view in cross-section of the two layers shown in Fig. 4 after the silver images have been transposed into dye images.

The undesired behaviour of photographic silver halide layers during the transformation into dye images and the manner in which it can be compensated for, are graphically illustrated in the attached drawing which refers to the above case where the dye images are obtained by local destruction of the dyes at the silver areas. Fig. 1 represents a photographic layer known in the prior art that is uniformly colored as indicated by horizontal hatching and contains a silver image of graded density, variations of the density being illustrated schematically by the vertically hatched steps in the drawing.

Fig. 2 employs the same graphical method to show the dye image left in such a prior art layer after the dye has been destroyed where silver was present, the silver being eliminated from the picture. The graduations recorded during the exposure and shown in Fig. 1 extend over a wide range but the dye image represented in Fig. 2 reproduces but a portion of these graduations. Fig. 3 illustrates graphically dye images obtained by other methods or under other processing conditions from silver pictures of the type illustrated in Fig. 1. In every case it is observed that the graduations of the dye image do not exactly reproduce the graduations of the original silver image or the original exposure and that details are lost in the conversion into dye images.

The present invention is intended to obviate the shortcomings above described and permits of dye images being obtained that reproduce the full range of graduations in better conformity with the range of light intensities originally recorded during the exposure. The principle upon which the invention is based is graphically illustrated in Fig. 4 in the same manner as employed in Figs. 1 to 3. Fig. 4 shows two light-sensitized layers of which layer A consists of a silver halide emulsion of the same nature as that in Fig. 1 and thus records the graduations of the exposure in the same manner. Layer B is immediately adjacent to layer A and in respect to the coloring both layers are substantially identical, the dye in layer B being employed in obtaining a color picture just as is the case with the dye in layer A. Layer B is also substantially identical with layer A in respect to the spectral sensitivity as both are intended to record the same color of the object. The only difference between the two

layers is that layer B is considerably less sensitive than layer A, the result being that while layer A records a broad range of light intensities, layer B records only the highest lights. This characteristic of layer B is illustrated in Fig. 4 which shows that only the greatest intensities of light recorded in layer A are also recorded in layer B.

Fig. 5 illustrates the material shown in Fig. 4 after the production of a dye picture and corresponds to Fig. 4 in the same manner as Fig. 2 to Fig. 1. The effect of the uniting of the two layers that are sensitized to different degrees in accordance with this invention is to be seen from the character of the finished dye picture graphically represented in Fig. 5. The range of light intensities which, although recorded by layer A in the form of a silver deposit is lost during the transformation into a dye image, is recorded by layer B in the form of a silver deposit of such lower densities that an image-like graduation of the dye is obtainable. Thus the details lacking in layer A appear as a dye image in layer B and both layers together reproduce the full range of the recorded light intensities.

The invention above described in principle may be realized in practice as illustrated in the following example:

Two silver halide layers, one of which consists of a highly sensitive panchromatic emulsion (sensitivity 28° Sch) while the other consists of an emulsion with a sensitivity of about 13° Sch, are coated in superposition on a support. Both emulsions are colored with 0.4 grm. per sq. m. Benzopurpurine 10B (Schultz Farbstofftabellen, Leipzig 1931, 7th ed., vol. 1, No. 489).

After exposure under a graduated wedge, the steps of which differ in density by 0.2 in logarithmic units and after treatment in a bath containing 5% hydrochloric acid, 15% sodium chloride and 0.01% 2-amino-3-oxyphenazine sulphonic acid, the highly sensitized emulsion layer yields a color picture the threshold of which corresponds with that of the silver image, but in which nevertheless only the lower 7 or 8 graduations of light are reproduced instead of the 15 steps recorded in the form of silver.

There are, however, a further 7 or 8 graduations reproduced in color by the less sensitive layer and thus the dye images in the two layers together reproduce the total scale recorded during exposure.

The double-layer of red-dyed emulsion may form a component of a multilayer material in which the other layers may also consist of double layers. For instance, the red-dyed double-layer described above may have superposed on it another double-layer composed, according to the principles outlined above, of a highly sensitive and a less sensitive orthochromatic emulsion each containing 0.6 grm. per sq. m. Chrysophenine G (Schultz I. c., No. 726). A surface layer in front of the two composite layers may be formed of an ordinary blue-sensitive emulsion that if required may be dyed after exposure.

In many cases it is preferable to have the layer of the less sensitive emulsion arranged nearer the source of light than the more highly sensitized layer of the same color. This is an advantage in certain circumstances, as instanced in the example cited above and in which there is a blue-sensitive layer in front of the double layer dyed yellow by Chrysophenine. In certain circumstances and especially when the absorption of the yellow dye present in the inner

layer is not too great, the blue light rays recorded in the blue-sensitive layer may penetrate into the yellow layer and produce a latent image therein that really ought only to be recorded in

5 the blue-sensitive layer. It is therefore advantageous if the surface of the yellow-dyed layer that is first hit by the blue light rays is not formed of the highly sensitive emulsion but rather of the emulsion with a relatively low sensitivity and which moreover is screened against blue light by the yellow dye.

Another advantage of the invention, independent of the relative position of the two layers, may be achieved by the invention when different 15 dyes of approximately the same shade are employed to dye the two parts of the composite layer. It is well known that various requirements must be taken into consideration when choosing the dyes suitable for the composition 20 of a color photograph, for instance, care must be taken that the dye does not affect the sensitivity too much, that it does not adversely affect the sensitizer, that it is or may be fixed in the layer so that it does not wash out or diffuse. 25 These considerations often result in the dye not having the shade that would be the most suitable for the production of a color photograph or for its behaviour when used as a master image in a further printing operation. In the event

30 of the dye in the highly sensitive layer not being perfectly adequate in respect to its absorption, it is possible to introduce a dye of similar shade into the less sensitive layer that, however, has better absorption properties than the dye in the 35 highly sensitive layer. The total absorption of the double layer is then the sum of the absorption of the two layers and better satisfies the demand for a faithful color reproduction or for good printing characteristics of the color photograph. Thus, for example, instead of coloring 40 each emulsion with 0.4 grm. per sq. m. Benzopurpurine 10B, only the highly sensitive emulsion is colored in this manner, whereas the emulsion of lower sensitivity is colored by means of 45 0.4 grm. per sq. m. Tuchechtrot 3B (Schultz Farbstofftabellen, Leipzig 1932, 7th ed., vol. 2, page 222). The total absorption of both layers together for light of the wave length  $510 \mu\mu$  is equal in both cases, whereas for light of the wave length  $410 \mu\mu$  Tuchechtrot 3B has a lower absorption than Benzopurpurine 10B and the sum of both absorptions is smaller than would be the case if both layers were dyed by Benzopurpurine 10B.

55 What is claimed is:

1. A light-sensitive photographic material for the production of colored images which comprises two superposed silver halide emulsion layers, each of said layers having evenly distributed therein 60 a coloring substance adapted to produce colored images of approximately the same color in both layers, both layers being sensitized to and transmittant for light of the same spectral composition, the one of said layers having a comparatively low speed with respect to the other layer.

2. A light-sensitive photographic material for the production of color images which comprises two superposed silver halide emulsion layers, each of said layers having evenly distributed therein 65 a dye adapted to produce colored images of approximately the same color in both layers, both layers being sensitized to and transmittant for light of the same spectral composition, the one of said layers having a comparatively low speed

with respect to the other layer, the said dyes being resistant to ordinary photographic treating solutions and capable of being bleached with the aid of metallic silver.

3. A light-sensitive photographic material for the production of color images which comprises two superposed silver halide emulsion layers, both layers being sensitized to and transmittant for light of the same spectral composition, the one of said layers having a comparatively low speed with respect to the other layer, and both layers being dyed with the same dye, said dye being resistant to ordinary photographic treating solutions and capable of being bleached with the aid of metallic silver.

4. A light sensitive photographic material for the production of colored images which comprises two superposed silver-halide emulsion layers, each of said layers having evenly distributed therein a coloring substance adapted to produce colored images of approximately the same color in both layers, both layers being sensitized to and transmittant for light of the same spectral composition, one of said layers being adapted to initially receive an optical image and having a comparatively low speed with respect to the other of said layers which is adapted to secondarily receive the optical image.

5. A light sensitive photographic material for the production of colored images which comprises two superposed silver-halide emulsion layers, both layers being sensitized to and transmittant for light of the same spectral composition, one of said layers having a comparatively low speed with respect to the other layer, each of said layers being dyed with dyes having different characteristics to that of the other layer but adapted to render substantially the same color, said dyes being resistant to ordinary photographic treating solutions and capable of being destroyed in the presence of metallic silver.

6. A photographic film comprising a transparent support, a fast light-sensitive silver-halide emulsion layer thereon, and a relatively slow light-sensitive silver-halide emulsion layer surrounding said fast emulsion layer, both of said layers being predominantly sensitive to and transmittant for light of the same spectral composition and containing coloring matter adapted to produce images of substantially the same color within both of said layers.

7. The method of producing a colored photograph of a desired range of different light intensities of an image field by a coloring process in which a photographic record produced within a light sensitive emulsion and representing said range of different light intensities is transformed to a colored image which reproduces in color a limited portion only of said range of different light intensities, which comprises forming in an emulsion layer sensitive to light of a predetermined spectral range a photographic record representing the desired range of different light intensities of the image field, forming in another superposed emulsion layer sensitive to light of the same spectral range a registering photographic record of said image field while restricting the response of said layer predominantly to a range of light intensities lost in the transformation of the photographic record in said first mentioned layer to a colored image by said coloring process, and transforming both of said photographic records into images of substantially the same color by said coloring process, whereby the range of light intensities reproduced in color in

said first mentioned layer is supplemented by the range of light intensities reproduced in color in said superposed layer.

8. The method of producing a colored photograph of a desired range of different light intensities of an image field by a coloring process in which a photographic record produced within a light sensitive emulsion and representing said range of different light intensities is transformed to a colored image which reproduces in color a limited portion only of said range of different light intensities, which comprises forming in an emulsion layer sensitive to light of a predetermined spectral range a photographic record representing the desired range of different light intensities of the image field, forming in a slower superposed emulsion layer sensitive to light of the same spectral range a registering photographic record representing predominantly those intensities of said image field that are not reproduced in color by the transformation of the record in said first mentioned layer to a colored image by said coloring process, and transforming both of said photographic records into images of substantially the same color by said coloring process.

9. The method of producing a colored photograph of a desired range of different light intensities of an image field by a coloring process in which a photographic silver image produced within a diffusely dyed light sensitive emulsion and representing said range of different light intensities is transformed to a colored image by local destruction of the dye at the places where silver is present, which comprises forming in a diffusely dyed emulsion layer sensitive to light of a predetermined spectral range a photographic silver image representing the desired range of different light intensities of the image field, forming in another superposed emulsion layer sensitive to light of the same spectral range and diffusely dyed with a dye of substantially the same color a registering photographic silver image of the same image field representing predominantly those light intensities of the image field that are recorded by the most opaque areas of the silver image in said first mentioned layer, treating both silver images simultaneously with a dye-destroying bath which is capable of destroying said dye locally with the aid of metallic silver, and removing the silver from the layers.

10. The method of producing a colored photograph of a desired range of different light intensities of an image field by a coloring process in which a photographic silver image produced within a diffusely dyed light sensitive emulsion and representing said range of different light intensities is transformed to a colored image by local destruction of the dye at the places where silver is present, which comprises forming in a diffusely dyed emulsion layer sensitive to light of a predetermined spectral range a photographic silver image representing the desired range of different light intensities of the image field, forming in another superposed emulsion layer sensitive to light of the same spectral range and diffusely dyed with the same dye as said first mentioned layer a registering photographic silver image of the same image field representing predominantly those light intensities of the image field that are recorded by the most opaque areas of the silver image in said first mentioned layer, treating both silver images simultaneously with a dye-destroying bath which is capable of destroying said dye locally with the aid of metallic silver, and removing the silver from the layers.

11. The method of producing a colored photograph correctly representing a desired range of different light intensities which comprises, recording an image representing a predetermined spectral range of an image field within a light-sensitive silver halide emulsion layer, recording a second image of the same image field representing the same spectral range within a second light-sensitive silver halide emulsion layer that is relatively faster than said first mentioned emulsion layer, developing silver images within said layers, and treating said layers to transpose said silver images into colored images of substantially the same color, said process including the combining of the colored image within said second layer in superposition and registry with the colored image in said first mentioned layer to correct for disproportional transition from sil-

ver to color of the desired range of different light intensities represented by the silver image in said first mentioned layer.

12. A light sensitive photographic material for the production of colored images which comprises at least three superposed silver halide emulsion layers, two of said layers located behind a third layer having evenly distributed therein a dyestuff for producing colored images of the same color in both layers, both layers being sensitized to and transmittant for light of the same spectral composition, said third layer being predominantly sensitive to and transmittant for light of a spectral composition absorbed by the dyestuff in said two layers, the front one of said two layers having a comparatively low speed with respect to the other one of said two layers.

PAUL GOLDFINGER.